

Patented Nov. 28, 1922.

## UNITED STATES PATENT OFFICE.

JOHN MURDOCH SKELLEY AND JAMES MERSON, OF BATTERSEA, LONDON, ENGLAND,  
ASSIGNORS TO CONTINUOUS REACTION COMPANY LIMITED, OF LONDON, ENGLAND.

## MANUFACTURE OF FERROMOLYBDENUM.

Application filed May 29, 1922. Serial No. 564,616.

No Drawing.

To all whom it may concern:

Be it known that we, JOHN MURDOCH SKELLEY and JAMES MERSON, both subjects of the King of Great Britain, residing at 155 5 Church Road, Battersea, London, England, have invented new and useful Improvements in the Manufacture of Ferromolybdenum, of which the following is a specification.

This invention relates to improvements in the manufacture of ferromolybdenum, i. e., alloys of molybdenum and iron in various proportions, containing up to about 85 per cent of molybdenum respectively.

These alloys have hitherto been manufactured as a rule from ores or mixtures containing iron and molybdenum by reduction either in the electric furnace or by the alumino-thermic process. In some cases the alumino-thermic reduction has been effected by means of a mixture of aluminium and ferrosilicon, but it has not been possible to dispense with the use of a substantial proportion of aluminium, which is a relatively costly reducing agent.

15. The present invention is based upon the discovery that if ores or mixtures containing iron and molybdenum in the form of oxides be mixed with pulverized silicon or ferrosilicon and a suitable oxidizing agent containing nitrogen such as sodium nitrate, but without aluminium, reaction may be initiated at a point in a cold or heated mixture as in the alumino-thermic process, and if suitable proportions of the ingredients be used the reaction proceeds to completion, ferromolybdenum practically free from carbon and silicon resulting.

According to this invention, therefore, ferromolybdenum is produced without the aid of aluminium by the silico-thermic reduction of a mixture of oxide of iron with oxide of molybdenum, or of an ore containing iron and molybdenum in the form of oxide, by means of silicon or ferrosilicon in the presence of a suitable oxidizing agent containing nitrogen, such as sodium nitrate or calcium nitrate.

As a rule, the richer the reducing agent is in silicon, the better is the reaction. Commercial silicon, which contains up to about 95% Si, or ferrosilicon containing from 99 to 70% Si, can be used with excellent results.

It will be understood that with ferrosilicon containing lower proportions of silicon the reaction becomes more sluggish and a limiting composition is reached which depends upon the method of working.

Commercial ores, with or without the addition of iron oxide, can be used for the purpose of the invention and are if necessary subjected to a preliminary treatment having for its object the removal of tin compounds, sulphur or other injurious matter such as arsenic or bismuth or an excess of silicious impurities, and conversion of all the iron and molybdenum into the form of oxide.

The following example illustrates the invention:

A molybdenum ore containing 80 per cent of  $MgS_2$  and 6 per cent of  $FeO$  is subjected to a preliminary purification to remove any bismuth present and is then treated to remove the sulphur. Of the product about 140 lbs. (containing 100 lbs.  $MoO_3$ ) are mixed with 20 lbs. of mill scale, 37 lbs. of ferrosilicon (90% Si) and 10 lbs. of sodium nitrate. Preferably 8 lbs. of calcium fluoride are added to enhance the fluidity of the slag. The mixture is put into a crucible and reaction is initiated as in the alumino-thermic process.

What we claim is:

1. The manufacture of ferromolybdenum without the aid of aluminium by the silico-thermic reduction of iron oxide and molybdenum oxide in the presence of an oxidizing agent containing nitrogen.

2. The manufacture of ferromolybdenum without the aid of aluminium by the silico-thermic reduction of iron oxide and molybdenum oxide in the presence of sodium nitrate.

3. The manufacture of ferromolybdenum by purifying the molybdenum ore to remove bismuth and sulphur, mixing the product with iron oxide, ferrosilicon and an oxidizing agent containing nitrogen and producing reaction as in the well known alumino-thermic process.

4. The manufacture of ferromolybdenum without the aid of aluminium by the silico-thermic reduction of iron oxide and molybdenum oxide in the presence of a nitrate oxidizing agent.

5. The manufacture of ferromolybdenum

by purifying the molybdenum ore to remove bismuth and sulphur, mixing the product with iron oxide, ferrosilicon and a nitrate oxidizing agent and producing reaction as in the well known alumino-thermic process.

6. The manufacture of ferromolybdenum by a silico-thermic reaction in a mixture of 140 parts purified molybdenum ore, 20 parts

of mill scale, 37 parts of ferrosilicon and 10 parts of sodium nitrate.

In testimony that we claim the foregoing as our invention we have signed our names this 17th day of May, 1922.

JOHN MURDOCH SKELLEY.  
JAMES MERSON.